

## UNITED STATES PATENT OFFICE

2,522,575

## FORGING ALUMINUM ALLOY

Horace Campbell Hall, Littleover, Harold Ernest Gresham, Little Eaton, near Derby, and William Michael Doyle and Clifford Wilson, Slough, England, assignors to Rolls-Royce Limited, Derby, England, a British company, and High Duty Alloys Limited, Slough, England, a British company

No Drawing. Application January 10, 1949, Serial No. 70,146. In Great Britain January 23, 1948

3 Claims. (Cl. 148—32.5)

1

This invention is for a new and improved way of producing wrought articles of aluminium alloy especially parts of internal combustion engines which have to resist high stresses at high temperatures.

It is known that silicon considerably facilitates the production of sound castings of aluminium alloys of the type which include copper, magnesium, nickel and iron.

Where an ingot must be cast in order to make the article in question especially a large ingot it is particularly desirable that blow holes and shrinkage cavities are to be avoided and a sound casting produced.

It is good foundry practice therefore to include at least 0.5 per cent of silicon to ensure a good casting.

We have found that the presence of silicon of this amount and more is however disadvantageous when the alloy is to be used at high temperatures, i. e. temperatures of the order of 200° C. and upwards. If, however, the alloy hereinafter described is to be produced by the ordinary chill cast or die cast methods silicon of the order of 0.5 per cent at least must be included to make casting practicable.

We have discovered that it is possible to make satisfactory forgings which have a low percentage of silicon and which achieve desirable properties at high temperature and to do so by initially selecting the elements of the alloy within narrow limits, casting the alloy in a special manner and giving it a particular heat treatment.

We have also found that articles made in this way have improved properties at room temperature.

According to this invention we make a forged article of aluminium base alloy by forming the alloy with the elements in the respective quantities hereunder mentioned, casting the ingot by the direct chill casting process, forging the same to the shape desired, and subjecting the same to the undermentioned heat treatment.

By "forging" we include any method of plastic deformation whether carried out hot or cold. If any considerable plastic deformation is required the process would be carried out at an elevated temperature.

The alloy is compounded of aluminium and the

following elements in the following proportions:

|           | Per cent    |
|-----------|-------------|
| Copper    | 1.8 to 2.5  |
| Magnesium | 1.2 to 2.0  |
| Nickel    | 0.8 to 1.5  |
| Iron      | 0.85 to 1.5 |

(but so that the combined content of iron and nickel does not exceed 2.75 per cent)

|    |          |             |
|----|----------|-------------|
| 10 | Silicon  | 0 to 0.4    |
|    | Titanium | 0.02 to 0.2 |

15 Niobium, cerium, beryllium, zirconium, antimony, manganese, molybdenum, chromium, vanadium, zinc, cobalt and silver may be added up to 0.5 per cent each, but not more than 1.5 per cent in total. The content of cobalt may be increased above 0.5 per cent up to 1 per cent if the nickel or the iron is correspondingly reduced

20 and the content of the silver above 0.5 per cent up to 1 per cent if the copper is correspondingly reduced. In each of which cases, the above mentioned maximum of 1.5 per cent may be correspondingly exceeded.

25 Calcium, barium and strontium should not be present in a total amount of more than 0.2 per cent. One or more of the following elements may be present up to a maximum of 0.1 per cent total: tin, arsenic, bismuth, cadmium, boron, lithium, sodium and potassium.

The heat treatment is to give solution treatment at 525 to 545° C. for from 2 to 30 hours, to quench and to age from 170° C. to 250° C. for from 1 to 30 hours. Quenching in boiling water may be advantageous.

30 This invention is particularly suitable for making parts of internal combustion engines which are of comparatively large size and are subject to stresses at high temperatures such as super-40 charge rotors of internal combustion engines of both the turbine and piston type, and pistons of the latter type of engine.

The alloy is particularly suitable for super-45 charge rotors of internal combustion turbines which are hot at their extremities but not at the centre where the stresses are highest.

The casting of the alloy is carried out by the direct chill casting process which may be either the continuous or semi-continuous process. In both of these processes, the molten metal is con-

## 3

tinuously poured at a controlled rate and temperature into a shallow water-cooled mould or die, where solidification commences. The die is of the required peripheral shape. At the same time, the ingot is continuously withdrawn through the bottom of the die, where the solidification is completed by jets of water or by immersion of the ingot in a tank full of water. In the continuous process, arrangements are made by means of a flying saw, or intermediate salt layers, or by interposed sheets of asbestos, or other suitable material, to separate the cast form into the desired ingot lengths, while the ingot is being continuously cast. On the other hand, the casting is intermittent in the case of the semi-continuous process. When the required ingot length has been cast, the pouring is temporarily suspended while the cast ingot is being removed.

Two alloys have been tested to show the comparative advantages of an alloy according to this invention.

Alloy A was formed according to this invention and was of the following composition:

|           | Per cent    |
|-----------|-------------|
| Copper    | 2.1 to 2.3  |
| Magnesium | 1.5 to 1.7  |
| Nickel    | 1.2 to 1.4  |
| Iron      | 1.0 to 1.3  |
| Silicon   | 0.15 to 0.2 |
| Titanium  | About 0.06  |

Alloy B was of the same composition but included silicon from 0.8 to 1.0 per cent.

Alloy A was produced by the semi-continuous casting process, forged and heat treated for 20 hours at 525-530° C., quenched in boiling water and aged 20 hours at 200° C.

Alloy B was produced by ordinary ingot casting methods, forged and heat treated for 20 hours at 520 to 525° C., quenched in boiling water and aged 20 hours at 170° C.

Both these heat treatments are the best known to us for the particular alloys and for the results desired.

#### Results of tensile tests

|                                                        | Alloy A | Alloy B |
|--------------------------------------------------------|---------|---------|
| Cold:                                                  |         |         |
| Max. Stress                                            | 28.7    | 27.2    |
| 0.1% Proof Stress                                      | 21.6    | 19.1    |
| Hot, tested at 300° C. after 1 hour at temperature:    |         |         |
| Max. Stress                                            | 10.3    | 9.6     |
| 0.2% Proof Stress                                      | 9.4     | 8.5     |
| Hot, tested at 300° C. after 100 hours at temperature: |         |         |
| Max. Stress                                            | 6.5     | 5.1     |
| 0.2% Proof Stress                                      | 4.6     | 3.9     |
| Hot, tested at 350° C. after 1 hour at temperature:    |         |         |
| Max. Stress                                            | 5.6     | 4.5     |
| 0.2% Proof Stress                                      | 5.0     | 3.4     |
| Hot, tested at 350° C. after 100 hours at temperature: |         |         |
| Max. Stress                                            | 3.5     | 2.6     |
| 0.2% Proof Stress                                      | 2.5     | 1.8     |

#### Creep tests

|              | Load, in tons per sq. in. | Percent Creep Strain   |                        |
|--------------|---------------------------|------------------------|------------------------|
|              |                           | Alloy A                | Alloy B                |
| Temperature: |                           |                        |                        |
| 200° C.      | 10                        | 0.15 [after 300 hours] | [0.22] after 300 hours |
| 225° C.      | 6½                        | 0.24 [after 300 hours] | 1.16 [0.23] hours      |
| 250° C.      | 3                         | 0.14 [after 300 hours] | [0.23] hours           |
| 300° C.      | 2                         | 0.61, after 209 hours  | 1.45, after 209 hours  |

#### Fatigue—Endurance rotating cantilever (based on 40 million reversals)

|                     | Alloy A, Tons per sq. in. | Alloy B, Tons per sq. in. |
|---------------------|---------------------------|---------------------------|
| Temperature 20° C.  | +10.5                     | +9.5                      |
| Temperature 200° C. | ±6.9                      | ±6.1                      |
| Temperature 300° C. | ±4.2                      | ±3.5                      |
| Temperature 350° C. | ±2.2                      | ±1.8                      |

10 The fatigue figures on Alloy A were characterized by a remarkable consistency in results.

15 Alloy A has further been tested after being produced by the same continuous casting process forged and solution treated for two hours at 545° C. quenched in boiling water and aged for one hour at 250° C. The following results were obtained at room temperature:

|                   | Tons per sq. in. |
|-------------------|------------------|
| 20 Maximum stress | 27.7             |
| 0.1% proof stress | 22.7             |

25 The same alloy solution treated for 20 hours at 525° C. quenched in boiling water and aged for 2 hours at 250° C. gave the following results:

|                   | Tons per sq. in. |
|-------------------|------------------|
| Maximum stress    | 27.1             |
| 0.1% proof stress | 20.6             |

30 That the improved results are not merely due to the method of casting is demonstrated by the following comparison. Two alloys C and D were made up within the range of composition given for alloy A and B respectively. Both alloys were cast by the semi-continuous casting process. They were then given the following heat treatment:

#### Heat treatment

35 Alloy C—  
2 hours at 530° C., quenched in water at 70° C., and aged for 20 hours at 200° C.

Alloy D—  
2 hours at 525° C., quenched in water at 70° C., and aged for 16 hours at 170° C.

45 The alloys were then forged into bar and subjected to the following tensile tests:

|                                         | Tensile Tests | Alloy C | Alloy D |
|-----------------------------------------|---------------|---------|---------|
| 50 Cold:                                |               |         |         |
| Max. Stress, tons per sq. in.           | 30.9          | 29.6    |         |
| 0.1% Proof Stress, tons per sq. in.     | 20.9          | 19.3    |         |
| Hot, Tested at 250° C. after 100 hours: |               |         |         |
| Max. Stress                             | 13.5          | 10.6    |         |
| 0.1% Proof Stress, tons per sq. in.     | 10.9          | 7.3     |         |
| Hot, Tested at 250° C. after 400 hours: |               |         |         |
| Max. Stress                             | 10.9          | 7.1     |         |
| 0.1% Proof Stress, tons per sq. in.     | 8.4           | 4.6     |         |

"Tons," as herein referred to, means long tons of 2,240 lbs. each.

46 What we claim is:

60 1. A forged aluminium alloy consisting by weight of 1.8% to 2.5% copper, 1.2% to 2.0% magnesium, 0.8% to 1.5% nickel, 0.85% to 1.5% iron, the iron and nickel together not exceeding 2.75%, up to and not exceeding 0.4% silicon, 0.02% to 0.2% titanium, and the balance essentially all aluminium substantially as described, said alloy being in the condition created by its having been subjected in the order stated to direct chill casting, forging, solution heat treating at 525° to 545° C. for 2 to 30 hours, quenching, and then ageing at 170° to 250° C. for 1 to 30 hours.

65 2. A forged aluminium alloy consisting by weight of 1.8% to 2.5% copper, 1.2% to 2.0% magnesium, 0.8% to 1.5% nickel, 0.85% to 1.5%

iron, the iron and nickel together not exceeding 2.75%, up to and not exceeding 0.4% silicon, 0.02% to 0.2% titanium, and the balance essentially all aluminium substantially as described, said alloy being in the condition created by its having been subjected in the order stated to direct chill casting, forging, solution heat treating at 525° to 545° C. for 2 to 30 hours, quenching, and then ageing at 170° to 250° C. for 1 to 30 hours, said alloy having a tensile strength of 10 approximately 6.5 tons per square inch after 100 hours at 300° C. and a fatigue endurance, measured by the rotating cantilever test based on 40 million reversals, of plus-and-minus approximately 4.2 tons per square inch at 300° C.

3. A forged aluminium alloy consisting by weight of 2.1% to 2.3% copper, 1.5% to 1.7% magnesium, 1.2% to 1.4% nickel, 1.0% to 1.3% iron, 0.15% to 0.2% silicon, about 0.06% titanium, and the balance essentially all aluminium substantially as described, said alloy being in

the condition created by its having been subjected in the order stated to direct chill casting, forging, solution heat treating at 525° to 530° C., quenching, and then ageing at 200° C.

HORACE CAMPBELL HALL.  
HAROLD ERNEST GRESHAM.  
WILLIAM MICHAEL DOYLE.  
CLIFFORD WILSON.

## REFERENCES CITED

The following references are of record in the file of this patent:

## UNITED STATES PATENTS

| 15 | Number    | Name              | Date          |
|----|-----------|-------------------|---------------|
|    | 1,744,545 | Hall et al. ----- | Jan. 21, 1930 |
|    | 2,022,686 | Nock, Jr. -----   | Dec. 3, 1935  |
|    | 2,087,988 | Nock, Jr. -----   | July 27, 1937 |
| 20 | 2,087,989 | Nock, Jr. -----   | July 27, 1937 |
|    | 2,381,714 | Beck -----        | Aug. 7, 1945  |